# EUROPEAN PATENT SPECIFICATION

(11) **EP 1 384 887 B1**
(45) Date of publication and mention of the grant of the patent: **27.07.2005**
(21) Application number: 03024463.6
(22) Date of filing: 08.05.1996
(51) Int. Cl.: F04B 27/08, F04B 27/10

(54) **Reciprocating compressor**
Kolbenkompressor
Compresseur à déplacement alternatif

(43) Date of publication of application: 28.01.2004
(62) Divisional of application: 96913701.7
(73) Proprietor: Kabushiki Kaisha Toyota Jidoshokki, Kariya-shi, Aichi-ken (JP)
(72) Inventor: Kato, Masafumi, Kariya-shi Aichi-ken (JP); Ito, Akichika, Kariya-shi Aichi-ken (JP)
(74) Representative: Leson, Thomas Johannes Alois, Dipl.-Ing.

(56) References cited:
- US-A- 4 519 119
- US-A- 5 056 417
- PATENT ABSTRACTS OF JAPAN vol. 011, no. 228 (M-610), 24 July 1987 (1987-07-24) & JP 62 041980 A (TAIHO KOGYO CO LTD;OTHERS: 01), 23 February 1987 (1987-02-23)
- PATENT ABSTRACTS OF JAPAN vol. 015, no. 358 (M-1156), 10 September 1991 (1991-09-10) & JP 03 141876 A (TOYOTA AUTOM LOOM WORKS LTD), 17 June 1991 (1991-06-17)
- PATENT ABSTRACTS OF JAPAN vol. 1997, no. 01, 31 January 1997 (1997-01-31) & JP 08 247026 A (TOYOTA AUTOM LOOM WORKS LTD), 24 September 1996 (1996-09-24)

## Description

### TECHNICAL FIELD

The present invention relates generally to a compressor (eg US-A-5056417) according to the preamble of claim 1.

### BACKGROUND ART

A reciprocating compressor, for example, as shown in Figure 10, is typically employed in air conditioners for automobiles and the like. This compressor has a pair of cylinder blocks 30 and 31 combined with each other. A swash plate chamber 32 is defined between these cylinder blocks 30 and 31. Housings 35 and 36 are attached to the outer end faces of the cylinder blocks 30 and 31 via valve plates 33 and 34, respectively. An intake chamber 36 and a discharge chamber 37 are defined between the valve plate 33 and the housing 35 and also between the valve plate 34 and the housing 36.

The drive shaft 39 is rotatably supported in these cylinder blocks 30 and 31. A swash plate 40 serving as a cam is fixed, in the swash plate chamber 32, to the drive shaft 39. A plural pairs of cylinder bores 41 and 42 are defined in the cylinder blocks 30 and 31 around the drive shaft 39. A double-headed piston 43 is housed in each pair of cylinder bores 41 and 42. Shoes 44, which serve as cam followers, are located between the swash plate 40 and each piston 43. Each shoe 44 has a sliding surface 45 that makes sliding contact with the front face or rear face of the swash plate 40 and a spherical surface 47 that makes sliding contact with a receiving recess 46 of the piston 43.

In the compressor described above, when the swash plate 40 is rotated with the rotation of the drive shaft 39, each piston 43 is reciprocated in the cylinder bores 41, 42 via the shoes 44 under the action of the swash plate 40. When the piston 43 is reciprocated, a refrigerant gas is introduced from the intake chamber 37 to the cylinder bores 41 and 42 as each piston 43 moves from the top dead center to the bottom dead center. Then, the refrigerant gas introduced into the cylinder bores 41 and 42 is compressed as the piston 43 moves from the bottom dead center to the top dead center and is discharged to the discharge chamber 38.

Generally, in order to increase the discharge capacity of a compressor, increasing the size of the cylinder bores 41 and 42 and increasing the sizes of the pistons 43, swash plate 40 and shoes 44 is contemplated. The pistons 43 and the swash plate 40 are generally made of a light aluminum alloy or the like. However, these members, which are made of the same metallic material, may seize. Accordingly, shoes 44 made of a ferrous metal are located between the pistons 43 and the swash plate 40 to prevent seizure between the pistons 43 and the swash plate 40. However, since ferrous metals have high specific gravity, the increase in the size of the shoes 44 increases the total weight of the compressor.

Assume that only the size of the pistons 43 and that of the swash plate 40 are increased, without changing the size of the shoes 44, in order to increase the discharge capacity. However, if the discharge capacity is increased, the load applied by the pistons 43 via the shoes 44 to the swash plate 40 is also increased. Accordingly, if the size of the shoes 44 remains unchanged, the load applied per unit area of the spherical surfaces 47 and that of the sliding surfaces 45 of the shoes 44 is increased. Consequently, the sliding resistance between the spherical surfaces 47 of the shoes 44 and the receiving recesses 46 defined in the pistons 43 and the sliding resistance between the sliding surfaces 45 of the shoes 44 and the swash plate 40 are increased.

If the sliding resistance between the spherical surfaces 47 of the shoes 44 and the receiving recesses 46 of the piston 43 is increased, the shoes 44 cannot move smoothly along the inner surfaces of the shoe retaining recesses 46. The shoes are moved by the swash plate 40 within the receiving recesses 46. If the shoes cannot move smoothly, the load applied between the sliding surfaces 45 of the shoes 44 and the swash plate 40 is increased, which further increase the sliding resistance between the sliding surfaces 45 of the shoes 44 and the swash plate 40.

In the compressor described above, a refrigerant gas is introduced from an external refrigerant circuit via the swash plate chamber 32 into the intake chamber 37. The refrigerant gas introduced into the swash plate chamber 32 cools each part in the swash plate chamber 32 and also prevents pulsation caused by the introduction of the refrigerant into the cylinder bores 41 and 42. However, R134a (CF3CH2F), which contains no chlorine, is employed as the refrigerant gas. This gas does not disrupt the stratospheric ozone layer. Chlorine is used as an extreme-pressure additive. An "extreme-pressure additive" is a substance that reacts with the surface of a metal and forms a metallic compound film to reduce frictional resistance.The refrigerant gas introduced into the swash plate chamber 32 washes off, by its own action, lubricant located on the surfaces of the swash plate 40 and other parts, so that lubrication between the shoes 44 and the pistons 43 and swash plate 40 is not easily achieved. In such cases, if chlorine, serving as the extreme-pressure additive, is not present in the refrigerant gas molecules, a great sliding resistance exists.

Therefore, it is an objective of the present invention to provide a reciprocating compressor that reduces the sliding resistance at the cam-piston joints.

### DISCLOSURE OF THE INVENTION

The object is achieved by the features of claim 1. The compressor according to the present invention has cylinder blocks containing cylinder bores. A drive shaft is rotatably supported in the cylinder blocks. A cam is attached to the drive shaft to be rotatable integrally therewith. A piston is slidably housed in the cylinder bores. A cam follower is slidably held between the piston and the cam. As the cam rotates, the piston is reciprocated via the cam follower. The piston is made of an aluminum or aluminum alloy matrix. The piston contains a receiving portion for slidably receiving the cam follower therein. A coating layer containing tin as a major component is formed at the receiving portion of the piston.

Therefore, according to the present invention, the coating layers formed at the receiving portions of the pistons reduce sliding resistance between the receiving portions of the pistons and the cam followers. Accordingly, even if a shortage of a lubricant occurs in the compressor, the cam followers can slide smoothly in the receiving portions of the pistons. Thus, the cam can move the cam followers with a small force. Consequently, the load acting between the cam followers and the cam can be reduced to decrease sliding resistance between them.

The compressor comprises: a cylinder block containing a cylinder bore; a drive shaft rotatably supported in the cylinder block; a cam attached to the drive shaft to be rotatable integrally therewith; a piston slidably housed in the cylinder bore; and a cam follower slidably interposed between the piston and the cam; the piston being reciprocated via the cam follower as the cam is rotated; the piston being made of an aluminum or aluminum alloy matrix and having a receiving portion for slidably receiving the cam follower therein, with a coating layer containing tin as a major component being formed at the receiving portion of the piston.

Further, the cam follower may made of a ferrous metal matrix and have a first sliding portion slidably retained in the piston and a second sliding portion to be brought into slide contact with the cam; at least one of the first sliding portion and the second sliding portion having a coating layer containing tin as a major component.

The compressor may comprise a piston having an outer circumference to be brought into slide contact with the inner circumference of the cylinder bore and the coating layer is also formed on the outer circumference of the piston.

The cam may have a sliding portion to be brought into slide contact with the cam follower, with a coating layer containing tin as a major component being formed at the sliding portion.

The cam further may have to be brought into slide contact with the second sliding portion of the cam follower, with a coating layer containing tin as a major component being formed at the sliding portion.

The mentioned coating layer may contain at least one metal selected from the group consisting of copper, nickel, zinc, lead and indium.

The cam follower may be a shoe having a spherical surface and the receiving portion of the piston is a recess which slidably receives the spherical surface of the shoe therein.

The coating layer may contain one kind of solid lubricant selected from the group consisting of a fluororesin powder, a molybdenum disulfide powder, a carbon powder and a boron nitride powder.

### BRIEF DESCRIPTION OF THE DRAWINGS

Figure 1 is an enlarged cross-sectional view of a pertinent portion of a swash plate type compressor according to a first embodiment of the present invention;
Figure 2 is a perspective view showing a piston in the first embodiment;
Figure 3 is an enlarged cross-sectional view of a pertinent portion of the piston;
Figure 4 is a graph showing measurement results of time until seizure that occurred with the first embodiment;
Figure 5 is an enlarged cross-sectional view of a pertinent portion of a swash-plate type compressor according to a second embodiment of the invention;
Figure 6 is a graph showing measurement results of time until seizure that occurred with the second embodiment;
Figure 7 is a cross-sectional view showing a wave cam type compressor according to another embodiment of the invention;
Figure 8 is an enlarged cross-sectional view of a pertinent portion of a cam follower according to another embodiment of the invention;
Figure 9 is an enlarged cross-sectional view of a pertinent portion of a swash plate according to another embodiment of the invention; and
Figure 10 is a cross-sectional view of a prior art swash-plate type compressor.

### BEST MODES FOR CARRYING OUT THE INVENTION

### (First embodiment)

A swash plate type compressor according to a first embodiment of the present invention will be described below referring to Figure 1 to Figure 4. It should be noted here that the mechanical construction of the compressor of the first embodiment is substantially the same as that of the compressor shown in Figure 10, which was described with reference to the prior art. Therefore, like or the same components as those in the compressor shown in Figure 10 are affixed with the same reference numbers, respectively, and a description of them will be omitted. Therefore, only differences from the compressor shown in Figure 10 will be described.

As shown in Figures 1 to 3, the compressor according to the first embodiment, unlike the compressor shown in Figure 10, each piston 1 has a coating layer 6 containing tin as a major component formed over its entire surface. Each piston 1 has a pair of receiving recesses 2 which slidably receive spherical surfaces of shoes 44.

The piston 1 consists of a main body 5 made of an aluminum or aluminum alloy matrix and a coating layer 6 formed over the entire surface of the main body 5. As the aluminum alloy, for example, an Al-Si alloy or an Al-Si-Cu alloy can be suitably employed. The main body 5 is preferably an aluminum alloy matrix containing hard particles. Such aluminum alloy is typified by an aluminum-high silicon alloy. The aluminum-high silicon alloy contains about 10 to 30 % by weight of silicon. If the aluminum-high silicon alloy has a silicon content not exceeding the level at which a eutectic mixture is formed, the silicon can be present in the form of eutectic silicon (i.e., the hard particles). In the first embodiment, the main body 5 of the piston 1 is made of a matrix of aluminum-high silicon alloy 4 containing 12 % by weight of silicon 3.

Incidentally, other materials containing hard particles include, an Al-Mn intermetallic compound, an Al-Si-Mn intermetallic compound, an Al-Fe-Mn intermetallic compound and an Al-Cr intermetallic compound, and these materials may be used as the matrix of the main body 5.

Further, in the first embodiment, the shoes 44 are made of SUJ2 material (a steel material for a high carbon content chromium bearing) specified by JIS, while the swash plate 40 is made of an aluminum-high silicon alloy.

The pistons 1 to be employed in the compressor of the first embodiment may be suitably selected, for example, from Examples 1 to 9 having various type of coating layers 6, respectively, as described below. Pistons 1 of Examples 1 to 9 will be described one by one. In Examples 1 to 9, the main bodies 5 of the pistons 1 are of the same structure, and the coating layers 6 have different compositions.

### (Example 1)

The piston 1 of Example 1 has a tin-copper eutectoid plating layer as the coating layer 6. This coating layer 6 is formed as follows. The entire main body 5 is immersed in an aqueous solution containing 6 % by weight of potassium stannate and 0.012 % by weight of copper gluconate maintained at 60 to 80 DEG C is to effect electroless plating on the surface of the main body 5. Subsequently, the main body 5 is taken out of the aqueous solution and rinsed. Thus, a eutectoid plating layer of tin and copper is formed as the coating layer 6 over the entire surface of the piston 1, including the receiving recesses 2, which contact the shoes 44. The coating layer 6 contains 97 % by weight of tin and 3 % by weight of copper and has a thickness of 1.2 µm.

### (Example 2)

The piston 1 of Example 2 has a tin-nickel eutectoid plating layer as the coating layer 6. Specifically, a eutectoid plating layer of tin and nickel is formed as the coating layer 6 over the entire surface of the piston 1 including the receiving recesses 2 by employing an aqueous solution containing 6 % by weight of potassium stannate and 0.005 % by weight of nickel chloride in the same manner as in Example 1. The coating layer 6 contains 98 % by weight of tin and 2 % by weight of nickel and has a thickness of 1 µm.

### (Example 3)

The piston 1 of Example 3 has a tin-zinc eutectoid plating layer as the coating layer 6. Specifically, a eutectoid plating layer of tin and zinc is formed as the coating layer 6 over the entire surface of the piston 1 including the receiving recesses 2 by employing an aqueous solution containing 6 % by weight of potassium stannate and 0.005 % by weight of zinc sulfate in the same manner as in Example 1. The coating layer 6 contains 97 % by weight of tin and 3 % by weight of zinc and has a thickness of 1 µm.

### (Example 4)

The piston 1 of Example 4 has a tin-lead eutectoid plating layer as the coating layer 6. Specifically, a eutectoid plating layer of tin and lead is formed as the coating layer 6 over the entire surface of the piston 1 including the receiving recesses 2 by employing an aqueous solution containing 6 % by weight of potassium stannate and 0.007 % by weight of lead sulfate in the same manner as in Example 1. The coating layer 6 contains 95 % by weight of tin and 5 % by weight of lead and has a thickness of 2 µm.

### (Example 5)

The piston 1 of Example 5 has a tin-indium eutectoid plating layer as the coating layer 6. Specifically, a eutectoid plating layer of tin and indium is formed as the coating layer 6 over the entire surface of the piston 1 including the receiving recesses 2 by employing an aqueous solution containing 6 % by weight of potassium stannate and 0.005 % by weight of indium sulfate in the same manner as in Example 1. The coating layer 6 contains 97 % by weight of tin and 3 % by weight of indium and has a thickness of 1µm.

### (Example 6)

The piston 1 of Example 6 has a plating layer containing only tin as the coating layer 6. Specifically, a plating layer of only tin is formed as the coating layer 6 over the entire surface of the piston 1 including the receiving recesses 2 by employing an aqueous solution containing 6 % by weight of potassium stannate in the same manner as in Example 1. The coating layer 6 has a thickness of 1.5 µm.

### (Example 7)

The piston 1 of Example 7 has, as the coating layer 6, a tin-copper eutectoid plating layer containing a fluororesin powder as a solid lubricant. Specifically, a eutectoid plating layer of tin and copper containing a fluororesin powder is formed as the coating layer 6 over the entire surface of the piston 1 including the receiving recesses 2 by employing an aqueous solution containing 6 % by weight of potassium stannate, 0.003 % by weight of copper gluconate and 1.0 % by weight of a fluororesin powder in the same manner as in Example 1. The coating layer 6 contains 99 % by weight of tin, 0.9 % by weight of copper and 0.1 % by weight of the fluororesin powder and has a thickness of 1.4 µm.

### (Example 8)

While the piston 1 of Example 8 has a tin-copper eutectoid plating layer like the coating layer 6 in Example I, the coating layer 6, which is formed by chemical plating treatment in the same manner as in Example 1, is subjected to heat treatment at a temperature of 150° C for one hour.

### (Example 9)

The piston 1 of Example 9 has a tin-copper-zinc eutectoid plating layer as the coating layer 6. Specifically, a eutectoid plating layer of tin, copper and zinc is formed as the coating layer 6 over the entire surface of the piston 1, including the receiving recesses 2, by employing an aqueous solution containing 6 % by weight of potassium stannate, 0.003 % by weight of copper gluconate and 0.003 % by weight of zinc sulfate in the same manner as in Example 1. The coating layer 6 contains 97 % by weight of tin, 1.5 % by weight of copper and 1.5 % by weight of zinc and has a thickness of 1.2 µm.

The present inventors performed the following test so as to confirm anti-seizure performance of compressors using the pistons 1 of Examples 1 to 9 respectively. In this test, the time until seizure between the swash plate 40 and the shoes 44 was measured while each compressor, which was incorporated into an automotive air conditioner, was operated under severe conditions (where no lubricant is present in the compressor). The compressors were operated in this test under the following conditions; intake pressure: -0.5 kg/cm², discharge pressure: 3 kg/cm², revolutions of the drive shaft 39: 1000 rpm. Further, the shoes 44 were made of an SUJ2 (JIS) material, and the swash plates 40 were made of an aluminum-high silicon alloy. Further, in carrying out this test, a compressor using pistons made only of an aluminum-high silicon alloy 4 containing 12 % by weight of silicon 3, i.e., pistons having no coating layer 6, was provided as a comparative example and tested in the same manner as described above.

Figure 4 is a graph showing the results of this test. The test results shown in Figure 4 demonstrate that seizure between the shoes 44 and the swash plates 40 takes much longer under severe use conditions in the compressors employing the pistons 1 of Examples 1 to 9 having the coating layers 6 compared with the compressor of the comparative example. In particular, the compressor incorporated with the pistons 1 of Example 1, each having a tin-copper eutectoid plating layer as the coating layer 6, shows the best anti-seizure performance.

As described above, in the first embodiment, a coating layer 6 containing tin as a major component is formed on the surface of each piston 1. Tin is a self-lubricating substance. Accordingly, sliding resistance between the receiving recesses 2 of the piston 1 and the spherical surfaces 47 of the shoes 44 is reduced, and even when there is a shortage of lubricant in the compressor, the shoes 44 can move smoothly along the inner surfaces of the receiving recesses 2. Accordingly, the swash plate 40 can move the shoes 44 within the receiving recesses 2 with a small force. As a result, the load acting between the sliding surface 45 of each shoe 44 and the swash plate 40 is moderated to reduce sliding resistance between the sliding surface 45 and the swash plate 40. Therefore, when the discharge capacity of a compressor is to be increased, even if the sizes of the pistons 1 and of the swash plate 40 are increased without increasing the size of the shoes 44, no problems arise due to an increase in the sliding resistance.

The coating layer 6 is formed over the entire surface of each piston 1. Accordingly, the sliding resistance between the outer circumference of the piston 1 and the inner circumferences of the cylinder bores 41 and 42 is reduced to allow smooth movement of the piston in the cylinder bores 41 and 42.

By incorporating at least one metal selected from copper, nickel, zinc, lead and indium in the coating layer 6 that contains tin as the major component, not only can the coating layer 6 be densified, but a hard metallic compound can be dispersed throughout the coating layer 6 to reinforce it. This reduces the coefficient of friction and abrasion resistance. For example, when copper is incorporated into the coating layer 6 that contains tin as the major component, the coating layer 6 is densified and a hard tin-copper compound (Cu₆Sn₅) is dispersed throughout the coating layer 6 to reinforce it.

The coating layer 6 is formed by means of chemical plating. With this chemical plating method, a eutectic mixture of tin and other metals, such as copper, can be easily deposited, and a solid lubricant, such as a fluororesin powder, can be easily incorporated into the coating layer 6.

### (Second embodiment)

Next, a swash plate type compressor according to a second embodiment of the invention will be described referring to Figures 5 and 6. It should be noted here that the mechanical constitution of the compressor of the second embodiment is substantially the same as that of the compressor shown in Figure 10 described referring to the prior art. Therefore, like or the same components as those in the compressor shown in Figure 10 are affixed with the same reference numbers respectively, and description of them will be omitted. Therefore, only the differences from the compressor shown in Figure 10 will be described.

As shown in Figure 5, the compressor according to the second embodiment, unlike the compressor shown in Figure 10, has shoes 7, each having a coating layer 11, containing tin as a major component, formed over its entire surface. The main body 12 of each shoe 7 is made of SUJ2 material as specified in JIS. The shoe 7 has a spherical surface 8 that slidably engages a receiving recess 46 of the piston 43 and a sliding surface 10, which makes sliding contact with the front face or rear face of the swash plate 40. The spherical surface 8 of the shoe 7 has a spherical portion 9 having a radius of curvature greater than that of the rest of the surface 8. An oil reservoir for storing a lubricant therein is defined between this spherical portion 9 and each receiving recess 46 of the piston 43. The sliding surface 10 of the shoe 7 is slightly tapered toward the periphery to have a convex-like shape to permit easy entry of lubricant into the clearance between the sliding surface 10 and the swash plate 40.

Further, in the second embodiment, both the swash plate 40 and the pistons 43 are made of an aluminum-high silicon alloy.

In the compressor of the second embodiment, suitable shoes 7 can be selected from those having various coating layers 11 as shown in the following Examples 1 to 9. The shoes 7 of Examples 1 to 9 will be described one by one. The main bodies 12 of the shoes 7 of Examples 1 to 9 are all the same, and only the coating layers 11 are different from one another.

### (Example 1)

The shoe 7 of Example 1 has a tin-copper eutectoid plating layer as the coating layer 11. This coating layer 11 is formed as follows. The main body 12 of the shoe 7 is immersed in an aqueous solution containing 6 % by weight of potassium stannate and 0.012 % by weight of copper gluconate. In this state, the main body 12 is connected to a cathode, and a metal bar having a high ionization tendency is used as an anode. When a predetermined voltage is applied between these electrodes using the thus prepared aqueous solution as an electrolyte, tin and copper are separated out under electrolytic action to adhere intimately to the surface of the main body 12. Subsequently, the main body 12 is taken out of the aqueous solution and rinsed. Thus, a eutectoid plating layer of tin and copper is formed as the coating layer 11 over the entire surface of the shoe 7.The shoe 7 thus plated is then surface polished while taking the clearance between the swash plate 40, with which the shoe 7 is used, and the piston 43 into consideration to have a uniform coating layer 11. The coating layer 11 contains 97 % by weight of tin and 3 % by weight of copper and has a thickness of 1.2µm.

### (Example 2)

The shoe 7 of Example 2 has a tin-nickel eutectoid plating layer as the coating layer 11. Specifically, a eutectoid plating layer of tin and nickel is formed as the coating layer 11 over the entire surface of the shoe 7 by employing an aqueous solution containing 6 % by weight of potassium stannate and 0.005 % by weight of nickel chloride in the same manner as in Example 1. The coating layer 11 contains 98 % by weight of tin and 2 % by weight of nickel, and the thickness of the coating layer 11 is adjusted to 1 µm by surface polishing.

### (Example 3)

The shoe 7 of Example 3 has a tin-zinc eutectoid plating layer as the coating layer 11. Specifically, a eutectoid plating layer of tin and zinc is formed as the coating layer 11 over the entire surface of the shoe 7 by employing an aqueous solution containing 6 % by weight of potassium stannate and 0.005 % by weight of zinc sulfate in the same manner as in Example 1. The coating layer 11 contains 97 % by weight of tin and 3 % by weight of zinc, and the thickness of the coating layer 11 is adjusted to 1 µm by surface polishing.

### (Example 4)

The shoe 7 of Example 4 has a tin-lead eutectoid plating layer as the coating layer 11. Specifically, a eutectoid plating layer of tin and lead is formed as the coating layer 11 over the entire surface of the shoe 7 by employing an aqueous solution containing 6 % by weight of potassium stannate and 0.007 % by weight of lead sulfate in the same manner as in Example 1. The coating layer 11 contains 95 % by weight of tin and 5 % by weight of lead, and the thickness of the coating layer 11 is adjusted to 2 µm by surface polishing.

### (Example 5)

The shoe 7 of Example 5 has a tin-indium eutectoid plating layer as the coating layer 11. Specifically, a eutectoid plating layer of tin and indium is formed as the coating layer 11 over the entire surface of the shoe 7 by employing an aqueous solution containing 6 % by weight of potassium stannate and 0.005 % by weight of indium sulfate in the same manner as in Example 1. The coating layer 11 contains 97 % by weight of tin and 3 % by weight of indium, and the thickness of the coating layer 11 is adjusted to 1 µm by surface polishing.

### (Example 6)

The shoe 7 of Example 6 has a plating layer containing tin only as the coating layer 11. Specifically, a plating layer of tin only is formed as the coating layer 11 over the entire surface of the shoe 7 by employing an aqueous solution containing 6 % by weight of potassium stannate in the same manner as in Example 1. The thickness of the coating layer 11 is adjusted to 1.5 µm by surface polishing.

### (Example 7)

The shoe 7 of Example 7 has a tin-copper eutectoid plating layer containing a molybdenum disulfide powder as a solid lubricant as the coating layer 11. Specifically, a eutectoid plating layer of tin and zinc containing the molybdenum disulfide powder is formed as the coating layer 11 over the entire surface of the shoe 7 by employing an aqueous solution containing 6 % by weight of potassium stannate, 0.003 % by weight of copper gluconate and 1.0 % by weight of the molybdenum disulfide powder in the same manner as in Example 1. The coating layer 11 contains 99 % by weight of tin, 0.9 % by weight of copper and 0.1 % by weight of the molybdenum disulfide powder, and the thickness of the coating layer 11 is adjusted to 1.4 µm by surface polishing.

### (Example 8)

While the shoe 7 of Example 8 has a tin-copper eutectoid plating layer as the coating layer 11 like in Example 1, the coating layer 11, which is formed by electrolytic plating treatment and polished in the same manner as in Example 1, is subjected to heat treatment at a temperature of 150° C for one hour.

### (Example 9)

The shoe 7 of Example 9 has a tin-copper-zinc eutectoid plating layer as the coating layer 11. Specifically, a eutectoid plating layer of tin, copper and zinc is formed as the coating layer 11 over the entire surface of the shoe 7 by employing an aqueous solution containing 6 % by weight of potassium stannate, 0.003 % by weight of copper gluconate and 0.003 % by weight of zinc sulfate in the same manner as in Example 1. The coating layer 11 contains 97 % by weight of tin, 1.5 % by weight of copper and 1.5 % by weight of zinc, and the thickness of the coating layer 11 is adjusted to 1.2 µm by surface polishing.

The present inventors performed the following test to confirm the anti-seizure performance of compressors using the shoes 7 of Examples 1 to 9, respectively. In this test, the time until seizure between the swash plate 40 and the shoes 7 was measured while each compressor, which was incorporated into an automotive air conditioner, was operated under severe conditions (where no lubricant is present in the compressor). The compressors were operated continuously in this test under the following conditions; intake pressure: -0.5 kg/cm², discharge pressure: 3 kg/cm², revolutions of the drive shaft 39: 1000 rpm. Further, the swash plates 40 and the pistons 43 of the compressors were made of an aluminum-high silicon alloy.Further, in carrying out this test, a compressor using shoes made of an SUJ2 material only, i.e., shoes having no coating layer 11, was provided as a comparative example and tested in the same manner as described above.

Figure 6 is a graph showing the results of this test. The test results shown in Figure 6 demonstrate that seizure between the shoes 7 and the swash plates 40 takes much longer under severe use conditions in the compressors employing the shoes 7 of Examples 1 to 9 having the coating layers 11 compared with the compressor of the comparative example. In particular, the compressor incorporated with the shoes 7 of Example 1, each having a tin-copper eutectoid plating layer as the coating layer 11, shows the best anti-seizure performance.

As described above, in the second embodiment, a coating layer 11 containing tin as a major component is formed on the surface of each shoe 7. Accordingly, sliding resistance between the receiving recesses 46 of the piston 43 and the spherical surfaces 8 of the shoes 7 is reduced, and the sliding resistance between the swash plate 40 and the sliding surface 10 of the shoe 7 is reduced. Accordingly, even when there is a shortage of lubricant in the compressor, smooth sliding of the swash plate 40 and the pistons 43 can be guarantied at the joints thereof to control sliding resistance at the joints.

The shoes 44 can move smoothly along the inner surfaces of the receiving recesses 46 under the action of the coating layer 11 formed on the spherical surfaces 8. As a result, the load acting between the sliding surface 10 of each shoe 7 and the swash plate 40 is moderated to reduce sliding resistance between the sliding surface 10 and the swash plate 40. The coating layer 11 is also present on the sliding surface 10 of the shoe 7, thus, the sliding resistance between the sliding surface 10 and the swash plate 40 can be further reduced. Therefore, when the discharge capacity of a compressor is to be increased, even if the sizes of the pistons 43 and the swash plate 40 are increased without changing the size of the shoes 7, no problems arise due to an increase in the sliding resistance.

Since tin not only exhibits excellent lubrication properties but also prevents rust, the coating layer 11 that contains tin as the major component formed on the surface of each shoe 7, which is made of a ferrous metal, can protect the shoe 7 from rusting.

Effects brought about by incorporating at least one metal selected from the group including copper to the coating layer 11 that contains tin as the major component are the same as in the first embodiment.

It should be understood that the present invention is not to be limited to the foregoing embodiments but may be embodied as follows by changing the make-up of the respective parts:
(1) In any of the first and second embodiments, while the present invention is embodied in a double-headed piston swash plate type compressor, the present invention may be embodied, for example, in a single-headed piston swash plate type compressor, a variable volume type compressor, which can adjust discharge volume by changing the tilt angle of the swash plate, a wave cam type compressor as shown in Figure 7, or the like. Incidentally, in the wave cam type compressor shown in Figure 7, like or the same components as those in the compressor shown in Figure 10 are affixed with the same reference numbers, respectively, and description of them will be omitted.As shown in Figure 7, this wave cam type compressor has a wave cam 48 having a wavy cam surface in place of the swash plate 40 in the compressor shown in Figure 1. The sliding surface 45 of each shoe 44 is designed to make sliding contact with the front cam surface or rear cam surface of the wave cam 48.
   In the wave cam type compressor described above, each piston 43 is adapted to reciprocate twice or more (twice in Figure 7) per revolution of the drive shaft 39, and the shoes 44 are required to follow the complicated cam surfaces as the cam surfaces produce displacement. Accordingly, in wave cam type compressors, compared with the swash plate type compressors, the conditions between the shoes 44 and the pistons 43 and between the shoes 44 and the wave cam 48 are more harsh. Accordingly, a reduction in the sliding resistance occurring at the junction of the wave cam 48 and the pistons 43 is important so that the wave cam type compressor can perform stable compression.
   In the compressor shown in Figure 7, to reduce sliding resistance occurring at the joints between the wave cam 48 and the pistons 43, the pistons 43 may be replaced with the pistons 1 as described in the foregoing first embodiment, or the shoes 44 may be replaced with the shoes 7 as described in the foregoing second embodiment.
(2) While substantially hemispherical shoes 7 and 44 were employed as cam followers in the first embodiment and the second embodiment, respectively, these shoes 77 and 44 may be replaced with a structure employing rollers. Otherwise, as shown in Figure 8, each cam follower may consist of a slipper 13, which makes sliding contact with the swash plate 40, and a ball 14, which engages a recess 13a of the slipper 13. The ball 14 is slidably engaged in the receiving recess 46 of the piston 43.Incidentally, in Figure 8, like or the same components as those in the compressor shown in Figure 10 are affixed with the same reference numbers, respectively, and descriptions of them will be omitted. In the construction shown in Figure 8, the pistons 43 may be replaced with the pistons 1 as described in the foregoing first embodiment, or the coating layer 11 as formed on the shoe 7 in the foregoing second embodiment may be formed on the slipper 13 or the ball 14 or both.
   The construction of the cam follower shown in Figure 8 may be applied to the above-described wave cam type compressor shown in Figure 7.
(3) In the first embodiment, a coating layer 15 that contains tin as the major component is formed on each surface of the swash plate 40, which makes sliding contact with the shoes 44, as shown in Figure 9. The composition of the coating layer 15 may be the same as that of the coating layer 6 of the piston 1. Thus, the sliding resistance between the swash plate 40 and the shoes 44 can be further reduced.
   A coating layer containing tin as the major component may be formed on the sliding surface 45 of each shoe 44 instead of forming the coating layers 15 on each side of the swash plate 40. In other words, the shoe 7 in the second embodiment may be given the coating layer 11 only at the sliding surface 10, and such shoes 7 may be employed as the shoes in the first embodiment.
(4) In the first embodiment, the coating layer 6 may be formed only at the receiving recesses 2 of the pistons 1.
(5) In the second embodiment, the coating layer 11 may be formed on either the spherical surface 8 or the sliding surface 10 of each shoe 7. When the coating layer 11 is formed only on the spherical surface 8 of the shoe 7, the coating layers 15 may be formed on each side of the swash plate 40 as described in (3).When the coating layer 11 is formed only on the sliding surface of the shoe 7, the piston 1 in the first embodiment, i.e., the piston 1 having the coating layer 6, may be employed.
(6) In the first embodiment, the surface of the main body 5 of the piston 1 may be subjected to pretreatment such as alumite treatment, manganese phosphate treatment, zinc phosphate treatment or zinc plating treatment prior to formation of the coating layer 6 on the main body 5. Thus, sliding resistance of the piston 1 with respect to the shoes 44 can further be reduced.
(7) In any of the foregoing embodiments, an alumina ceramic (Al2O3) layer may be formed on the sliding surface 10 of the main body 12 of each shoe 7 and the sliding surface 45 of each shoe 44.Thus, the sliding resistance of the shoes with the swash plate 40 can further be reduced.
(8) In any of the foregoing embodiments, the ratio of tin to other metals also present in the coating layer 6 or 11 may be suitably changed depending on the desired performance of the compressor. For example, when both tin and copper exist in the coating layer 6 or 11, the content of copper is desirably changed to within the range of 0.1 % by weight to 50 % by weight. If the content of copper is smaller than 0.1 % by weight, densification and reinforcement of the coating layer 6 or 11 cannot be fully achieved, and the effect to be brought about by incorporation of copper cannot be achieved. If the content of copper is greater than 50 % by weight, the self-lubricating action of tin cannot be fully achieved, which results in increased sliding resistance.
(9) In any of the foregoing embodiments, the fluororesin powder or the molybdenum disulfide powder incorporated in the coating layer 6 or 11 as a solid lubricant may be replaced with a carbon powder, a boron nitride powder, or the like.
(10) In any of the foregoing embodiment, the coating layer 6 or 11 may not be formed by means of wet plating process such as electrolytic plating and chemical plating but may be formed utilizing a CVD method or a dry plating method such as vacuum deposition, sputtering, ion plating and PVD. When the solid lubricant described in (9) is incorporated into the coating layer 6 or 11, a composite plating method may be employed.
(11) In any of the foregoing embodiments, the thickness of the coating layer 6 or 11 may be suitably adjusted in the range of 1 to 5 mu m. If the coating layer 6 or 11 has a thickness of smaller than 1 mu m, the coefficient of friction cannot be sufficiently reduced. If the coating layer 6 or 11 has a thickness greater than 5 mu m, a problem is likely to occur in the rigidity of the layer, and the coating layer 6 or 11 may separate.

## Claims

1. A compressor, comprising:
a cylinder block (30,31) containing a cylinder bore (41,42);
a drive shaft (39) rotatably supported by the cylinder block (30,31);
a cam (40,48) attached to the drive shaft (39) to be rotatable integrally therewith;
a piston (1, 43) housed in the cylinder bore (41,42); and
a shoe (7, 44) having a spherical and flat sliding surfaces and slidably interposed between the piston (1, 43) and the cam (40, 48);
the piston (1, 43) being reciprocated via the shoe (44) as the cam (40,48) is rotated;
the piston (1, 43) being made of an aluminum or aluminum alloy matrix and having a receiving recess (2, 46) for slidably receiving the spherical surface (8, 47) of the shoe (7, 44) therein, **characterized in that**
the shoe (7, 44) is made of a ferrous metal matrix; and
a coating layer (6) containing tin as a major component is formed at the receiving recess (2) of the piston (1).

2. The compressor according to claim 1,
**characterized in that**
a coating layer is formed at both of spherical and flat surfaces of the shoe (7).

3. The compressor according to Claim 1, wherein
the piston (1) has an outer circumference to be brought into slide contact with an inner circumference of the cylinder bore (41, 42), and the coating layer (6) is also formed on the outer circumference of the piston (1).

4. The compressor according to Claim 1, **characterized in that** a coating layer (6) is formed on the cam (40, 48) that reduces a sliding resistance between the cam (40, 48) and the shoe (7).

5. The compressor according to Claim 4, wherein the coating layer (6, 11) of the cam (40, 48) contains tin as its major component.

6. The compressor according to Claim 1 or 2, wherein a thickness of the coating layer (6, 11) is in a range of 1 to 5µm.

7. The compressor according to Claim 1 or 2, wherein the coating layer (6, 11) contains at least one component selected from a group consisting of copper, nickel, zinc, lead and indium.

8. The compressor according to Claim 1 or 2, wherein the coating layer (6, 11) contains one kind of solid lubricant selected from a group consisting of a fluororesin powder, a molybdenum disulfide powder, a carbon powder and a boron nitride powder.

9. The compressor according to claim 1, wherein tetrafluoroethane is used as a refrigerant gas.

## Patentansprüche

1. Kompressor mit:
einem eine Zylinderbohrung (41, 42) enthaltenden Zylinderblock (30, 31);
einer drehbar in dem Zylinderblock (30, 31) gelagerten Antriebswelle (39);
einer an der Antriebswelle (39) angebrachten Nocke (40, 48), um mit dieser zusammen gedreht zu werden;
einem in der Zylinderbohrung (41, 42) aufgenommenen Kolben; und
einem eine kugelige und flache Gleitfläche aufweisenden und gleitbar zwischen dem Kolben (1, 43) und der Nocke (40, 48) eingefügten Schuh (7, 44);
wobei der Kolben (1, 43) über den Schuh (44) hin- und herbewegt wird, wenn die Nocke (40,48) gedreht wird;
der Kolben (1, 43) aus einem Aluminium oder einer Aluminumlegierungsmatrix hergestellt ist und eine Aufnahmeaussparung (2, 46) aufweist, um die kugelige Oberfläche (8, 47) des Schuhs (7, 44) gleitbar darin aufzunehmen, **dadurch gekennzeichnet, dass**
der Schuh (7, 44) aus einer Eisenmetallmatrix hergestellt ist; und
eine Ummantelungsschicht (6), die Zinn als Hauptbestandteil enthält, bei der Aufnahmeaussparung (2) des Kolbens (1) ausgebildet ist.

2. Kompressor nach Anspruch 1,
**dadurch gekennzeichnet, dass**
eine Ummantelungsschicht sowohl bei der kugeligen als auch der flachen Oberfläche des Schuhs (7) ausgebildet ist.

3. Kompressor nach Anspruch 1, wobei der Kolben (1) einen äußeren Umfang aufweist, der in Gleitkontakt mit einem inneren Umfang der Zylinderbohrung (41, 42) zu bringen ist, und die Ummantelungsschicht (6) ebenfalls auf dem äußeren Umfang des Kolbens (1) ausgebildet ist.

4. Kompressor nach Anspruch 1, **dadurch gekennzeichnet, dass** eine Ummantelungsschicht (6) auf den Nocke (40, 48) ausgebildet ist, die einen Gleitwiderstand zwischen der Nocke (40, 48) und dem Schuh (7) reduziert.

5. Kompressor nach Anspruch 4, wobei die Ummantelungsschicht (6, 11) der Nocke (40, 48) Zinn als deren Hauptbestandteil enthält.

6. Kompressor nach Anspruch 1 oder 2, wobei eine Dicke der Ummantelungsschicht (6, 11) sich in einem Bereich von 1 bis 5 µm befindet.

7. Kompressor nach Anspruch 1 oder 2, wobei die Ummantelungsschicht (6, 11) zumindest einen Bestandteil enthält, der aus einer Gruppe ausgewählt wurde, die aus Kupfer, Nickel, Zink, Blei und Indium besteht.

8. Kompressor nach Anspruch 1 oder 2, wobei die Ummantelungsschicht (6, 11) eine Art eines festen Schmiermittels enthält, das aus einer Gruppe ausgewählt wurde, die aus einem Fluorharzpulver, eine Molybdendisulfitpulver, einem Kohlenstoffpulver und einem Bornitritpulver besteht.

9. Kompressor nach Anspruch 1, wobei Tetrafluorethan als Kältemittelgas verwendet wird.

## Revendications

1. Compresseur comprenant :
un bloc-cylindres (30, 31) contenant un alésage de cylindre (41, 42) ;
un arbre d'entraînement (39) supporté, pour tourner, par le bloc-cylindres (30, 31) ;
une came (40, 48) fixée sur l'arbre d'entraînement (39) pour pouvoir tourner en une seule pièce avec celui-ci ;
un piston (1, 43) logé dans l'alésage de cylindre (41, 42) ;
un patin (7, 44) présentant des surfaces coulissantes plate et sphérique, et intercalé, pour coulisser, entre le piston (1, 43) et la came (40, 48) ;
le piston (1, 43) étant animé d'un mouvement de va et vient, par l'intermédiaire du patin (44) lorsque la came (40, 48) tourne ;
le piston (1, 43) étant composé d'une matrice d'aluminium ou d'un alliage d'aluminium et présentant un évidement de réception (2, 46) afin de recevoir, par coulissement, la surface sphérique (8, 47) du patin (7, 44), à l'intérieur de celui-ci, **caractérisé en ce que**
le patin (7, 44) est composé d'une matrice d'un métal ferreux ;
une couche de revêtement (6) contenant de l'étain comme composant principal est formée au niveau de l'évidement de réception (2) du piston (1).

2. Compresseur selon la revendication 1, **caractérisé en ce qu'**une couche de revêtement est formée à la fois sur la surface sphérique et sur la surface plate du patin (7).

3. Compresseur selon la revendication 1, dans lequel le piston (1) présente une circonférence extérieure qui doit être amenée en contact coulissant avec une circonférence intérieure de l'alésage de cylindre (41, 42) et la couche de revêtement (6) est également formée sur la circonférence extérieure du piston (1).

4. Compresseur selon la revendication 1, **caractérisé en ce qu'**une couche de revêtement (6) est formée sur la came (40, 48) ce qui réduit une résistance au coulissement entre la came (40, 48) et le patin (7).

5. Compresseur selon la revendication 4, dans lequel la couche de revêtement (6, 11) de la came (40, 48) contient de l'étain comme composant principal.

6. Compresseur selon la revendication 1 ou 2, dans lequel une épaisseur de la couche de revêtement (6, 11) se trouve dans une fourchette comprise entre 1 et 5 µm.

7. Compresseur selon la revendication 1, dans lequel la couche de revêtement (6, 11) contient au moins un composant choisi dans un groupe consistant en le cuivre, le nickel, le zinc, le plomb et l'indium.

8. Compresseur selon la revendication 1 ou 2, dans lequel la couche de revêtement (6, 11) contient une sorte de lubrifiant solide choisi dans un groupe consistant en une poudre de fluororésine, une poudre de bisulfure de molybdène, une poudre de carbone et une poudre de nitrure de bore.

9. Compresseur selon la revendication 1, dans lequel le tétrafluroéthane est utilisé comme gaz réfrigérant.
